

## 1

2,901,886

**METHOD OF INCREASING ENGINE THRUST**

Mona Phyllis Doerner, Walnut Creek, Calif., assignor to The Dow Chemical Company, Midland, Mich., a corporation of Delaware

No Drawing. Application March 21, 1956  
Serial No. 572,805

7 Claims. (Cl. 60—35.4)

This invention relates to a novel and improved method of obtaining thrust from an engine capable of burning a high energy fuel. More particularly, it relates to a method of increasing the thrust of a rocket, jet or turbo-jet engine by supplying to the combustion zone of such an engine an improved high energy fuel.

Several materials have been used in the past as high energy fuels for rocket and jet engines. The term "high energy fuel" refers to fuels which spontaneously ignite and violently burn when mixed with an oxidizing agent such as hydrogen peroxide, nitric acid or nitrogen tetroxide to produce thrust in a rocket, jet or turbo-jet engine. High energy fuels frequently used in such engines include hydrazine, hydrazine hydrate, aniline and aliphatic hydrocarbons. A particular disadvantage of such fuels has been their liquidus properties whereby they freeze at temperatures commonly encountered in missile and jet plane flight. Another disadvantage of many such fuels has been their inability to produce high thrusts due to their unfavorable heats of combustion or undesirable ignition characteristics. A fuel which would be characterized by a high heat of combustion, low freezing point, short ignition delay and high specific impulse would be of outstanding value in the development of rockets and missiles. It is thus clearly evident that fuels having improved ignition, combustion and liquidus properties would be a distinct advantage to the development of the rocket and jet engine industry.

One object of this invention is to provide a novel method of obtaining thrust from an engine capable of burning a high energy fuel. Another object is to provide an improved method of increasing the thrust of an engine which burns a high energy fuel by supplying to the combustion zone of such an engine a fuel having very desirable liquidus, ignition and combustion properties. Other objects will appear throughout the following description and appended claims.

This new and improved method of providing thrust to an engine which will burn a high energy fuel will be more fully described hereinafter and the novelty thereof will be particularly pointed out and distinctly claimed.

In accordance with the present invention, it has been discovered that thrust may be obtained from an engine capable of burning a high energy fuel by supplying to the combustion zone of such an engine a propynyl compound having the general formula:



where R is hydrogen, methyl, ethyl or 2-propynyl and R<sub>1</sub> is amino, methyl or allyl, along with an oxidizer such as nitric acid, nitrogen tetroxide, hydrogen peroxide or oxygen. These propynyl compounds have very desirable overall characteristics such as high heat of combustion, high specific impulse, wide liquidus range and

## 2

short ignition delay whereby they are particularly adapted to be employed as high energy fuels. The compounds are stable liquids in air at normal temperatures and pressures. (2-propynyl) hydrazine and 1,1-bis (2-propynyl)

- 5 hydrazine freeze at approximately -60° C. and -45° C. and boil at 63°-66° C. at 17 millimeters pressure and 61°-63° C. at 4 millimeters pressure, respectively. Dimethyl (2-propynyl) amine and allyl di(2-propynyl) amine freeze at approximately -44° C. and -60° C. 10 respectively. The compounds also possess much higher heats of combustion than hydrazine as shown in the table below in which the heat of combustion is expressed in kilocalories per pound:

| Compound:                           | Heat of combustion |
|-------------------------------------|--------------------|
| Hydrazine                           | 1930               |
| (2-propynyl) hydrazine              | 3540               |
| 1,1-bis (2-propynyl) hydrazine      | 4020               |
| 1-methyl-1-(2-propynyl) hydrazine   | 3780               |
| 20 1-ethyl-1-(2-propynyl) hydrazine | 3930               |
| Methyl di(2-propynyl) amine         | 4440               |
| Dimethyl (2-propynyl) amine         | 4330               |
| Allyl di(2-propynyl) amine          | 4480               |

- 25 When operating in accordance with the present invention, the propynyl compound and the oxidizing agent are separately metered into the combustion chamber of the engine where combustion and violent burning take place spontaneously. In such operations, it is desirable that 30 the oxidizing agent be introduced into the combustion chamber at a rate and in an amount sufficient to effect substantially complete combustion of the propynyl fuel compound. The rate at which thrust is developed in the engine varies directly with the rate at which the 35 propynyl compound and oxidizing agent are metered into the combustion chamber. The propynyl compound may be supplied to the combustion zone along with other additives such as aniline, substituted anilines or aliphatic hydrocarbons. The thrust developed from the combustion of the fuel is found to be considerably greater when one or more of the propynyl hydrazines or propynyl amines is used as the fuel than when hydrazine is used. Since the thrust developed in an engine is directly proportional to the heat of combustion of the fuel employed, it is evident that an engine burning a propynyl hydrazine or propynyl amine can propel a missile proportionately further or can propel a proportionately greater load than an engine burning a conventional fuel.

The propynyl hydrazine and propynyl amine compounds used as fuels in the method of the present invention to increase engine thrust may be prepared by reacting propargyl bromide or propargyl chloride with hydrazine, methyl hydrazine, ethyl hydrazine, methylamine or allylamine. The reaction is carried out in an inert organic solvent such as a lower alcohol or diethyl ether. The reaction is exothermic and takes place smoothly at -10° to 80° C. with the production of the desired product and the hydrohalide of the hydrazine or amine reagent. Good results are obtained when employing one molecular proportion of propargyl halide with at least two molecular proportions of the hydrazine or amine reagent. Upon completion of the reaction, the desired product may be separated by fractional distillation under reduced pressure.

65 In accordance with the patent statutes, this invention has been fully and completely described including what is now considered to be one of its best embodiments. However, it will be apparent to those skilled in the art that other variations are possible. Thus, it should be understood that within the scope of the appended claims 70 this invention may be practiced otherwise than as specifically described.

What I claim is:

1. In a method of obtaining thrust from an engine adapted for producing thrust upon combustion therein of a high energy fuel with an oxidizer which will effect a hypergolic and spontaneous combustion with the fuel, and wherein the fuel and an amount of the oxidizer sufficient to effect substantially complete combustion thereof are simultaneously supplied to the combustion zone of said engine, the improvement which comprises employing as the high energy fuel a member of the group consisting of (2-propynyl) hydrazine, 1,1-bis(2-propynyl) hydrazine, 1-methyl-1-(2-propynyl) hydrazine, 1-ethyl-1-(2-propynyl) hydrazine, methyl di(2-propynyl) amine, di-methyl(2-propynyl) amine, and allyl di(2-propynyl) amine. 10

2. A method according to claim 1 in which the compound supplied to the combustion zone is (2-propynyl) hydrazine. 15

3. A method according to claim 1 in which the compound supplied to the combustion zone is 1,1-bis(2-propynyl) hydrazine.

4. A method according to claim 1 in which the compound supplied to the combustion zone is 1-methyl-1-(2-propynyl) hydrazine.

5. A method according to claim 1 in which the com-

20 pound supplied to the combustion zone is dimethyl (2-propynyl) amine.

6. A method according to claim 1 in which the compound supplied to the combustion zone is allyl di(2-propynyl) amine.

7. A method of increasing the thrust of an engine capable of burning a high energy fuel which comprises separately supplying to the combustion zone of said engine a high energy fuel with an amount of oxidizer sufficient to effect substantially complete combustion of the fuel, the high energy fuel being selected from the group consisting of (2-propynyl) hydrazine, 1,1-bis (2-propynyl) hydrazine, 1-methyl-1-(2-propynyl) hydrazine, 1-ethyl-1-(2-propynyl) hydrazine, methyl di(2-propynyl) amine, dimethyl (2-propynyl) amine and allyl di(2-propynyl) amine, and the oxidizer being selected from the group consisting of nitric acid, nitrogen tetroxide, hydrogen peroxide and oxygen.

20

References Cited in the file of this patent:

UNITED STATES PATENTS

2,573,471 Malina et al. Oct. 30, 1951  
2,712,496 Skolnik et al. July 5, 1955